

## UNITED STATES PATENT OFFICE

HAROLD J. KERSTEN, OF CINCINNATI, OHIO, ASSIGNOR TO BOARD OF DIRECTORS OF THE  
UNIVERSITY OF CINCINNATI, OF CINCINNATI, OHIO

## ELECTRODEPOSITION OF TIN-GOLD ALLOYS

No Drawing.

Application filed February 20, 1930. Serial No. 430,135.

The object of my invention is to produce deposits of white gold comprising primarily gold and tin, which deposits are suitable for use in the jewelry art and respond to the accepted jeweler's test for "gold",—i. e. which are not attacked by concentrated and dilute nitric acid.

Another object of my invention is the provision of an electrolytic bath and a treatment suitable for the control of such deposits. These and other objects of my invention which will be set forth herein-after or will be apparent to one skilled in the art upon reading these specifications, I accomplish by that certain procedure and in that article of which I shall now describe a preferred embodiment.

In the practice of my invention I employ an electrolyte comprising salts of gold and of tin. The bath may contain alkali cyanides of gold, together with alkali stannates, alkali stannites, salts to increase the conductivity, to produce buffer action, to alter the degree of dissociation of the gold and tin salts, and organic or inorganic compounds for the purpose of preventing decomposition of the other constituents of the bath.

In particular, I have found the following bath to produce satisfactory deposits:

Gold potassium cyanide (KAu(CN)<sub>2</sub>) 3 gm.  
Potassium stannate K<sub>2</sub>SnO<sub>3</sub>·3H<sub>2</sub>O 10 gm.  
Water 1 liter

as hereinabove indicated, the composition of my bath and the electric conditions under which it is used may be varied, all without departing from the scope of my invention.

Having thus described my invention, what I claim as new and desire to secure by Letters Patent, is:

1. A homogeneous dense electro-deposit of white gold comprising tin and gold as its major constituent, the said deposit being unattacked by nitric acid.

2. An electroplating bath for producing white gold comprising a cyanide salt of gold and a tin salt of an alkali metal, in water solution, the relative proportion of gold to tin in said electrolyte being low.

3. An electrolytic bath for depositing white gold comprising an alkali cyanide of gold and a tin salt, in water solution, the relative proportion of gold to tin in said electrolyte being low.

4. An electrolyte for depositing white gold comprising an alkali cyanide of gold and an alkali salt of stannic acid, in water solution, the relative proportion of gold to tin in said electrolyte being low.

5. A process for producing white gold electro-deposits, comprising, employing an electrolyte containing a gold salt and a tin salt, the relative proportion of gold to tin in the electrolyte being low, and plating from said electrolyte with an insoluble anode and a current density around one ampere per square centimeter.

6. An electrolyte for producing white gold deposits having substantially the following proportions:

Gold potassium cyanide (KAu(CN)<sub>2</sub>) 3 gm.  
Potassium stannate K<sub>2</sub>SnO<sub>3</sub>·3H<sub>2</sub>O 10 gm.  
Water 1 liter

HAROLD J. KERSTEN.

35 The composition and color of the alloy deposited may be altered by changing the current density, the size of the anode, and the temperature of the bath, the hydrogen ion concentration of the bath, the proportions of the components and the amount of agitation given to the bath during the electrodeposition. By way of example I may employ this bath with or without other ingredients at a temperature of 70° centigrade, a current density of one ampere per square centimeter, and an insoluble anode with or without agitation, and this procedure will give satisfactory white deposits which are dense and unattacked by concentrated and dilute nitric acid. For various purposes,